

## UNITED STATES PATENT OFFICE

2,455,554

## ELECTRODEPOSITION OF COPPER

Henry Brown, Detroit, Mich., assignor to The Udylite Corporation, Detroit, Mich., a corporation of Delaware

No Drawing. Application January 5, 1946,  
Serial No. 639,412

6 Claims. (Cl. 204—52)

1

This invention relates to the electrodeposition of copper from an acid bath.

The object of this invention is to decrease the grain size and increase the lustre of the copper deposit without materially impairing the ductility of the plate or decreasing the current density range of the copper plating bath.

I have found that this object can be accomplished by the addition of small concentrations of acetyl cyanamide



to standard acid copper plating baths.

This compound used in small concentrations in the acid copper sulfate bath (made up of simply copper sulfate and sulfuric acid) will cause the deposit obtained to be very brilliant. It will also decrease the grain size and increase the lustre of the copper plate obtained from the acidic copper fluoborate bath.

With the use of 0.1—0.7 g./l. of acetyl cyanamide brilliant ductile copper plate can be obtained from the simple acid copper sulfate bath. The composition of the bath may vary over wide limits, though for the highest rate of brightening and for the widest bright plating range, it is best not to use concentrations of sulfuric acid of much over 80 g./l. The standard acid copper plating baths of the compositions given by:

|                                           | Grams per liter |
|-------------------------------------------|-----------------|
| $\text{CuSO}_4 \cdot 5\text{H}_2\text{O}$ | 150 to 250      |
| $\text{H}_2\text{SO}_4$                   | 10 to 75        |

give very good results, though less copper sulfate and less acid may be used.

The following acidic copper plating baths can be used with improved results in smoothness and brightness by the addition of about 0.1 to 0.7 g./l. of acetyl cyanamide:

## Example A

|                                           | Grams per liter |
|-------------------------------------------|-----------------|
| $\text{CuSO}_4 \cdot 5\text{H}_2\text{O}$ | 200             |
| $\text{H}_2\text{SO}_4$                   | 10-25           |

## Example B

|                                           | Grams per liter |
|-------------------------------------------|-----------------|
| $\text{CuSO}_4 \cdot 5\text{H}_2\text{O}$ | 150             |
| $(\text{NH}_4)_2\text{SO}_4$              | 10-50           |
| $\text{H}_2\text{SO}_4$                   | 10-20           |

## Example C

|                                              | Grams per liter |
|----------------------------------------------|-----------------|
| $\text{Cu}(\text{BF}_4)_2$ copper fluoborate | 100-150         |
| Free $\text{HBF}_4$                          | 5-25            |

## Example D

|                          | Grams per liter |
|--------------------------|-----------------|
| $\text{CuBF}_4$          | 100-150         |
| $\text{NH}_4\text{BF}_4$ | 10-50           |
| $\text{HBF}_4$           | 1-25            |

2

It is best to operate the baths cold (50°—60° F.) or at room temperatures or below approximately 100° F. Higher temperatures decrease the rate of brightening and the bright plating range (the lower current density areas are dull). Too high concentrations of acid do likewise.

For the highest rate of brightening and the widest bright plating range, besides a low temperature, the use of vigorous agitation of the solution or cathode agitation is necessary. The use of such agitation besides enhancing the brilliance makes the copper ion concentration even less critical and also makes possible the use of high cathode current densities (100 amp./ft.<sup>2</sup> and higher) at which brilliant plate is obtained and also makes possible the use of higher anode current densities. The highest rate of brightening is obtained at the higher current densities.

A preferred bath from the standpoint of economy is:

|                                           | Grams per liter |
|-------------------------------------------|-----------------|
| $\text{CuSO}_4 \cdot 5\text{H}_2\text{O}$ | 150-200         |
| $\text{H}_2\text{SO}_4$                   | 10-25           |
| Acetyl cyanamide                          | 0.1-0.5         |

Temperature 50-75° F. Vigorous agitation of the bath or cathode. Cathode C. D. of 10-100 amp./ft.<sup>2</sup>.

The addition of ammonium sulfate at concentrations of 10-50 g./l. widens the bright plate range toward the lower current densities, though it does decrease somewhat the rate of brightening at the very highest current densities.

The addition of small amounts (0.005 to 0.1 g./l.) of gelatin or partially hydrolyzed gelatin or partially hydrolyzed gelatin or peptones improves the brightness further but decreases the ductility.

Acetyl cyanamide is a definite improvement over cyanamide or dicyandiamide, in that the bright plate range is wider, and there is less tendency for ribbing effects at the higher concentrations of brightener. Also for a given degree of brightness the plates are more ductile.

I claim:

1. A bath for electrodepositing bright copper comprising an aqueous acid copper solution comprising essentially a material selected from the group of materials consisting of copper fluoborate, a mixture of copper sulfate and sulfuric acid, a mixture of copper sulfate, ammonium sulfate and sulfuric acid, a mixture of copper fluoborate and hydrofluoboric acid, and a mixture of copper fluoborate, ammonium fluoborate and hydrofluoboric acid, said aqueous acid copper solution also having dissolved therein acetyl cyanamide in a concentration ranging from about .1 to .7 gram per liter, said bath having a temperature falling within a range of from about 50° F. to about 100° F. and containing a greater molar concentration of copper salt than of acid.

2. A bath for electrodepositing bright copper comprising an aqueous acid copper solution comprising essentially copper sulfate in a concentration falling within a range of from about 150 grams per liter to about 200 grams per liter and sulfuric acid in a concentration falling within a range of from about 10 grams per liter to about 25 grams per liter and having dissolved therein acetyl cyanamide in an amount falling within a range of from about .1 gram per liter to about .7 gram per liter, said bath having a temperature falling within a range of from about 50° F. to about 100° F.

3. A bath for electrodepositing bright copper comprising an aqueous acid copper solution comprising essentially copper fluoborate in a concentration falling within a range of from about 100 grams per liter to about 150 grams per liter and hydrofluoboric acid in a concentration falling within a range of from about 5 grams per liter to about 25 grams per liter and having dissolved therein acetyl cyanamide in an amount falling within a range of from about .1 gram per liter to about .7 gram per liter, said bath having a temperature falling within a range of from about 50° F. to about 100° F.

4. The method of electrodepositing bright copper comprising the step of electrodepositing copper from an aqueous acid copper solution having dissolved therein a material selected from the group of materials consisting of copper fluoborate, a mixture of copper sulfate and sulfuric acid, a mixture of copper sulfate, ammonium sulfate and sulfuric acid, a mixture of copper fluoborate and hydrofluoboric acid, and a mixture of copper fluoborate, ammonium fluoborate and hydrofluoboric acid, said aqueous acid copper solution also having dissolved therein acetyl cyanamide in a concentration ranging from about .1 to .7 gram per liter, said bath having a temperature falling within a range of from about 50° F. to about 100° F. and containing a greater molar concentration of copper salt than of acid.

5. The method of electrodepositing bright copper comprising the step of electrodepositing copper from an aqueous acid copper solution having dissolved therein a material selected from the group of materials consisting of copper sulfate, ammonium sulfate and sulfuric acid, a mixture of copper sulfate and hydrofluoboric acid, and a mixture of copper sulfate, ammonium sulfate and hydrofluoboric acid, said aqueous acid copper solution also having dissolved therein acetyl cyanamide in an amount falling within a range of from about .1 to .7 gram per liter, said bath having a temperature falling within a range of from about 50° F. to about 100° F. and containing a greater molar concentration of copper salt than of acid.

6. The method of electrodepositing bright copper comprising the step of electrodepositing copper from an aqueous acid copper solution comprising essentially copper sulfate in a concentration falling within a range of from about 150 grams per liter to about 200 grams per liter and sulfuric acid in a concentration falling within a range of from about 10 grams per liter to about 25 grams per liter and having dissolved therein acetyl cyanamide in an amount falling within a range of from about .1 gram per liter to about .7 gram per liter, said bath having a temperature falling within a range of from about 50° F. to about 100° F.

per comprising the step of electrodepositing copper from an aqueous acid copper solution comprising essentially copper sulfate in a concentration falling within a range of from about 150 grams per liter to about 200 grams per liter and sulfuric acid in a concentration falling within a range of from about 10 grams per liter to about 25 grams per liter and having dissolved therein acetyl cyanamide in an amount falling within a range of from about .1 gram per liter to about .7 gram per liter, said bath having a temperature falling within a range of from about 50° F. to about 100° F.

6. The method of electrodepositing bright copper comprising the step of electrodepositing copper from an aqueous acid copper solution comprising essentially copper fluoborate in a concentration falling within a range of from about 100 grams per liter to about 150 grams per liter and hydrofluoboric acid in a concentration falling within a range of from about 5 grams per liter to about 25 grams per liter and having dissolved therein acetyl cyanamide in an amount falling within a range of from about .1 gram per liter to about .7 gram per liter, said bath having a temperature falling within a range of from about 50° F. to about 100° F.

HENRY BROWN.

#### REFERENCES CITED

The following references are of record in the file of this patent:

#### UNITED STATES PATENTS

| Number    | Name   | Date          |
|-----------|--------|---------------|
| 2,164,924 | Hull   | July 4, 1939  |
| 2,374,289 | Hull   | Apr. 24, 1945 |
| 2,391,289 | Beaver | Dec. 18, 1945 |

#### OTHER REFERENCES

Modern Electroplating, special volume published by the Electrochemical Society, (1942), page 157.